

June 23, 1942.

B. J. OAKES

2,287,060

METHOD OF MAKING WATERPROOF SANDPAPER

Original Filed March 10, 1933



Patented June 23, 1942

2,287,060

# UNITED STATES PATENT OFFICE

2,287,060

## METHOD OF MAKING WATERPROOF SANDPAPER

Byron J. Oakes, St. Paul, Minn., assignor to  
Minnesota Mining & Manufacturing Company,  
St. Paul, Minn., a corporation of Delaware

Application March 10, 1933, Serial No. 660,318  
Renewed March 1, 1940

7 Claims. (Cl. 51—300)

This invention relates, in general, to the preparation of abrasive articles, preferably in sheet form, and more particularly to the treatment of sheet material for obtaining or forming composite structures in the form of abrasives, such as far example that which is commonly known as sandpaper. Composite structures of the abrasive type, such as sandpaper or emery cloth comprise generally—

(a) A base or backing of sheet material which may be felted, such as in the case of paper, or woven material, as in the case of cloth;

(b) A more or less finely comminuted resistant material having abrading properties, such as garnet, corundum, pulverized glass, and generally, natural and artificial abrasive materials; and

(c) A binder, generally in the form of an adhesive material, which serves to bind the abrasive to the base.

Where I have attempted to make abrasive products suitable for liquid sanding operations and having a high order of flexibility, in which the binding ingredients for the abrasive particles include the water repellent properties of materials of the general resinous type or resin-varnish type, including waterproofing materials such as oils, and utilize these materials in connection with the abrasive and the backing material to obtain an abrasive article having uniform properties of flexibility, thickness in connection with a predetermined size of the grit of abrasive particles, and abrasion resistance during operation for the life of the abrasive article, the application of the binder and the abrasive particles to a backing material such as paper, involves a number of perplexing problems due to the characteristics of the binding material, and the abrasive to react and make intimate contact with the binder; the nature of the reaction of the binder material or waterproofing ingredients in connection with the paper, the relative adjustment of the quantity of binder to the particles of grit or abrasive, to give abrading characteristics without clogging, all of which affect the uniformity of the product, the life of the abrasive article as to its abrasive characteristics, flexibility and resistance to the liquids used in abrading operations, such as water, solutions of detergents and organic solvents, such as kerosene, gasoline and oil.

While the problems above enumerated, when giving consideration to the materials entering into making the composite comprising sandpaper, by reason of the characteristics of the backing material, usually comprising paper or cloth, the bond for the abrasive particles of waterproofing material and the reaction of this bond to the backing material when in association with the abrasive particles, in themselves are very complex, the economical practice of such process is

extremely vital, and the success or failure of the industry engaged in the production of waterproof sandpaper depends upon its ability to obtain all the benefits above enumerated with certainty, uniformity and economy.

It is therefore an object of my invention to provide a waterproof sandpaper which includes the production of such material in which the characteristics of waterproofness, resistance to decomposition by liquids used in abrading operations, with uniformity of product as to maximum abrading efficiency and with prolonged abrasive life, coupled with flexibility, may be economically practiced and with certainty of results.

It is also an object of my invention to provide an improved process of manufacturing sandpaper and the like abrasive articles in which the backing is conducted through the various steps of application of sizing adhesive, binder adhesive and grit in such manner that, subsequent to the application of grits to the adhesive and while the sheet or backing having the grit thereon is passed through drying and heat-treating steps, the grit coated side of the sheet is maintained free of external mechanical pressure so as to prevent dulling of the sheet and thus produce an article in which the sharper edges of the abrading grits are presented at the abrading surface.

It is also contemplated as an object of my invention to provide an adjustment of the constituents of the waterproofing materials and volatile vehicle used therefor comprising, generally, resinous and oily constituents whereby the various steps of application of the coats comprising the presize for the backing, the binder coat for the grit, the backsize and the sand-size, will permit the sheet carrying these coatings to pass through the drying and heat-treating steps with great speed and facility so that the coatings quickly take on sufficient rigidity whereby the sheet may be handled without external mechanical pressure which would otherwise be necessary to render the constituents of the binder homogeneous and, which if applied, would disturb the abrasive particles and present a duller working abrading surface.

A still further object of my invention resides in the provision of waterproofing compositions, serving as sizing or binder coats in the production of waterproof and flexible sandpaper of value in the practice of the methods hereinbefore referred to, assuring the economical and uniform production of waterproof and flexible sandpaper of the maximum abrading efficiency.

For the attainment of the aforementioned objects and for such other objects as may appear herein or may be hereinafter pointed out, and for a clearer understanding of the method contemplated by my invention, reference will now

be made to the accompanying drawing forming a part hereof, in which the Figures 1 and 1a are diagrammatic illustrations of the sandpaper making process in accordance with my invention.

In this view, a backing material 10 is provided in the form of a continuous sheet and is fed to printing rolls 11 for the proper identification of the sandpaper to indicate the grade of paper or for the application of a trade mark and similar notations. From the printing roll, the backing is then fed to pressure transfer rolls 12 whereby a presize is affixed to one surface of the paper. The web so treated is then festooned through festooning racks 13 to aerate the backing carrying the presize. Immediately thereafter, the web is then passed through a surface coating apparatus in the nature of pressure rolls 14 for transferring to the surface to which the presize has been applied, a film of a binder coat. The web is then immediately passed to an abrasive sprinkling apparatus 15 so that the abrasive is deposited with the binder coat in a still tacky condition. The web is then reflexly bent at 16 so that excess abrasive particles are discarded and permitted to fall freely from the surface of the web. The fabric carrying the sizing coat, binder coat and abrasive is then passed over a festooning rack 17 after which the web is passed through an oven 18 having suitable festooning racks.

I find it desirable that the sheet or backing material 10, after receiving the grit layer from the hopper 15 and while passed through the festooning steps indicated at 17 and through the oven, as indicated at 18, to so conduct the backing that the grit coated side thereof is maintained out of direct contact with pressure rolls so that from the time of application of the grit until the adhesive is substantially fully set, passing from the chamber 20 of the oven 18, the grits do not become dulled or materially disturbed and thus, when the finished article is rolled upon the making roll 21, the adhesive is sufficiently set so as to prevent turning over the grits from a predetermined deposited position so that a relatively large number of the grits will be presented with their sharper cutting edges outwardly.

Where the paper is carried through the secondary step of the operation, as hereinafter described, I also, in this instance, maintain the sheet out of contact with the pressure rolls, with the exception of the point at which the sand sizing coat may be applied if desired.

I find that I am able to avoid direct contact with pressure rolls which may disturb the desirable position of the abrasive particles, by reason of the character and nature of the waterproofing composition that I use and which will be more particularly referred to hereinafter, constituting the copolymerized and reaction product of resinous materials, particularly a "phenol-fatty-oil-reactive resin" and a "fatty oil" in a volatile vehicle. The homogeneity of this product and the speed with which it sets and matures enables me to handle the web in the manner hereinbefore described. The oven is divided into chambers 19 and 20, respectively, the first of which is heated at a relatively high temperature, and the second of which maintains a temperature materially lower than the first chamber. Up to this point, the webbing may be said to have been going through the making process, and may thereafter be formed into a roll 21 to await treatment for finishing by sizing.

However, the making process may be followed immediately by the sizing in a continuous operation, and for this purpose, the web may then be passed through pressure transfer rolls 22, where a film of back-size is applied to the surface of the webbing opposite to that carrying the abrasive particles. The webbing thus treated may then be passed through festooning racks 23, and then immediately passed through pressure transfer rolls 24, where a film of a sandsize is applied to the grit surface of the web so prepared. The web then passes through ovens 25 and 26 respectively, the first of which is maintained at a higher temperature, the second of which is maintained at a relatively lower temperature. In these ovens, as well as the ovens previously mentioned at 19 and 20, means are provided to control the humidity within the ovens to about 38%.

From the oven 26, the composite sheet so prepared is first subjected to a mist of water by the spraying device 28 sprayed on the back-size in quantities just sufficient, so that the paper does not cockle, from which point, the composite is then formed into a roll 29 to await suitable treatment subsequently by cutting the same into small sheets, disks, rolls or other forms for the market.

For the continuous operation briefly above referred to, in connection with the diagrammatic illustration of the process, to attain the objectives heretofore mentioned, reference will now be made to the details of the process briefly described above.

The success of the process involves a proper relationship of the backing material to the size in order to afford a proper preliminary preparation of the paper for the subsequent treatment, and to permit of a continuous operation which will produce uniformity of results. The paper

webbing, where this form of backing material is used, is so chosen, as well as the consistency of the sizing composition and method of applying it, to assure a continuous film upon the backing of minimum penetration, yet of definite uniformity.

For this purpose, with a sizing material of the character to be described and the method of application to be described, I provide a paper stock which has an oil absorption factor of thirty-five minutes, made by the Fourdrinier method.

The sizing composition and the method of applying it are so controlled as to give a continuous film of about six to 12 grains per square foot, and for this purpose, pressure rolls whereby the fluid sizing coat has transferred to it the sizing material, are utilized at the point 12 above referred to.

In my preferred form of the invention, a sizing coat of the following formula is used:

#### Example A

|                             | Per cent |
|-----------------------------|----------|
| China-wood oil              | 23.06    |
| Aluminum stearate           | 1.85     |
| 53 Rosin                    | 4.36     |
| Lime                        | .20      |
| Manganese oxide             | .012     |
| Litharge                    | .023     |
| Lead acetate                | .108     |
| 70 Cobalt acetate           | .027     |
| Oleum spirits               | 64.34    |
| Blanc fixe (barium sulfate) | 4.99     |
| Turpentine                  | 1.03     |

This formula in relation to the paper backing

of the character above referred to, is most suitable for my purposes. The paper should be a hard, tinny sheet without shiny spots and as free as possible from such defects as slime spots, dark spots, wrinkles and cockels. The utilization of a sizing coating of the character described, is characterized by a relationship of the waterproofing ingredients and body imparting resins, comprising the China-wood oil and rosin respectively, and the solvent comprising oleum spirits and turpentine, in that in the subsequent evaporation of the solvent by the air drying process over the festoons 13 the waterproofing ingredients will remain in perfect solution to the end point of evaporation of the thinners, assuring a uniformity of film and sufficient viscosity to prevent segregation of the solid mineral materials, including the organic and inorganic driers. The mineral materials included are characterized by their compatibility with the paper backing, avoiding undue penetration of the extremely thin film of sizing material, so that a continuous film is provided, cooperating with the backing to provide an extremely flexible product.

Following the application of a sizing coat, the web passes over the festooning racks 13 so as to evaporate by aeration, the solvent of the sizing coat. The surface exposure of the festooning racks is such that within a period of about thirty-five minutes, the web has completely passes over the racks, and the presize coat is now in condition for having applied thereto the binder coat.

In accordance with the apparatus heretofore described, the binder coat is applied by pressure rolls 14, one of the rolls of the series being dipped into a tank including the binder composition, provision being made for heating this binder composition to a temperature of about 160 degrees F.

The binder coat is transferred to the size surface of the backing to obtain the requisite film, in accordance with the size of grit to be used. For grits of a mesh of 60 to 120, the following binder coat compositions may be used:

*Example B*

|                      | Per cent |
|----------------------|----------|
| China-wood oil       | 24.4     |
| Rosin                | 4.07     |
| Lime                 | .13      |
| Manganese oxide      | .29      |
| Litharge             | .08      |
| Kauri                | 12.2     |
| Ester gum            | 6.5      |
| Linseed oil (boiled) | 27.53    |
| Oleum spirits        | 10.5     |
| Wood turpentine      | 14.3     |

*Example C*

|                           |       |
|---------------------------|-------|
| China-wood oil            | 60.0  |
| Phenol formaldehyde resin | 19.8  |
| Linseed oil               | .13   |
| Rosin                     | .006  |
| Lime                      | .001  |
| Litharge                  | .002  |
| Cobalt acetate            | .001  |
| Turpentine                | 19.93 |
| Oleum spirits             | .13   |
| Manganese oxide           | Trace |

Immediately following the application of the binder coat by the method described, the abrasive particles are sprinkled over the binder coat, preferably heating the grit to a temperature of about 100 degrees F.

The relationship of the mixed resins and gums

to the solvents which characterizes the formulas above enumerated as B and C constituting the essential features of my invention, particularly in relation to the abrasive particles and to the sizing material initially deposited upon the backing, is the ability of the thinner to maintain the ingredients in perfect solution at all times up to the end point of evaporation, notwithstanding the wetting effect the binder may have upon the grit or abrasive particles, or the capillary attraction caused by contacting particles of grit. The binder coat in relation to the sizing coat is further characterized by anchorage to the sizing coat without re-solution to an extent as will cause penetration of the sizing coat into the backing material with the consequent starving of the binder coat.

For grits of a fineness of from 220 to 400 mesh, I may increase the fluidity of the binder coat by the addition of a greater amount of thinners in percentage of about 15% for 220 mesh and 25% for 400 mesh. At all times, this percentage and the character of thinners used is such that the oils and resins and soluble materials, where organic driers are used, are such that the materials will be kept in solution without segregation and to the end point of evaporation of the thinners, even where baking temperatures are used to evaporate the thinners. The mixed thinners used are further characterized by the fact that the entire solution wets the abrasive, and under the influence of the wetting action of the abrasive particles, the mixed thinners which are used are characterized by complete solution of the organic materials used in the thinners up to the end point of evaporation.

It will further be observed that the character of binder coat used in relation to the sizing coat and the treatment given to the sizing coat will result in a predetermined thickness or depth of film being formed upon the sizing coat to leave a film of binder which anchors the grit to a predetermined depth and to properly expose the abrading edges. This relationship of the binder coat to the sizing coat is particularly important with the finer mesh grits, to assure proper abrading efficiency with adequate anchoring of these particles.

Following the application of the binder coat and grit, the webbing carrying the materials are festooned as described over the festooning racks 17 for a short period to initially remove some of the thinners. The web then passes into the oven 18 at the compartment 19 over racks included therein in number sufficient to pass through the compartment 19 within a period of two hours. The compartment 19 is maintained at a temperature of about 175 degrees F., provision being made to draw off such volatile vapors as may be generated by reason of the thinners that are used.

The passage of the web through the compartment 19 is for such period of time so that at the temperature used, the relative position of the grit in the binder coat will not be modified, and further, the abrading efficiency of the grit will not be modified. The temperature to which the web is then exposed in passing through the compartment 20 is materially reduced to approximately 140 degrees F. The extent of the rack surfaces maintained within the compartment 20 is such as to prolong this compartment for a period of about twenty-eight hours. At the end of this period of time, the binder has been thoroughly matured and as previously described, the web

may be formed into the roll 21 to be stored for subsequent use in the sizing operations.

The web, however, may be fed continuously to the applicator 22 which includes pressure transfer rolls, at which point a composition as follows may be applied to the back of the web as a back-size, the composition being as follows:

*Example D*

|                           | Per cent |    |
|---------------------------|----------|----|
| China wood oil            | 21.8     | 10 |
| Boiled linseed oil        | 7.25     |    |
| East India (resin)        | 7.3      |    |
| Cobalt acetate            | 0.2      |    |
| Oleum spirits             | 36.0     |    |
| Gilsonite                 | 3.57     | 15 |
| Beyerlite                 | 0.71     |    |
| Eocene (petroleum source) | 4.2      |    |
| Water                     | 13.4     |    |
| Alum                      | 0.85     |    |
| Soap                      | 1.18     | 20 |
| Isinglass                 | 1.18     |    |
| Alcohol                   | 2.36     |    |

The composition under Example D is maintained at a temperature of about 130 degrees F. This formula under the method of application is characterized by sufficient fluidity to form a continuous film by its further property of being anchored to the backing material at the back surface without impregnation to an extent as would alter the first sizing coat by striking through to the front face of the backing. The formula and the method of application are further characterized by compatibility with the backing, to result in a film which will resist decomposition by the liquids used in abrading operations, yet offering sufficient frictional characteristics at the back surface.

After application of the formula in accordance with Example D, the webbing is air-dried by passing the web over festooning racks 23 for a period of about thirty-five minutes. The web then passes through the applicator in the nature of pressure transfer rolls 24, at which point the sandsize is applied to the grit surface.

At this point, a composition in the nature of following is applied:

*Example E*

|                 | Per cent |    |
|-----------------|----------|----|
| China wood oil  | 35.2     | 50 |
| Rosin           | 5.41     |    |
| Ester gum       | 7.11     |    |
| Lime            | 0.18     |    |
| Manganese oxide | 0.05     |    |
| Litharge        | 0.10     | 55 |
| Lead acetate    | 0.03     |    |
| Turpentine      | 6.67     |    |
| Oleum spirits   | 45.25    |    |

However, I may use, for the sandsize, a composition as follows:

*Example F*

|                                                |       |    |
|------------------------------------------------|-------|----|
| China wood oil                                 | 37.5  |    |
| Phenol formaldehyde resin (oil reactive resin) | 12.35 | 65 |
| Linseed oil                                    | .08   |    |
| Resin                                          | .004  |    |
| Lime                                           | Trace |    |
| Litharge                                       | .001  | 70 |
| Cobalt acetate                                 | .001  |    |
| Turpentine                                     | 50.0  |    |
| Manganese oxide                                | Trace |    |

The sand size is maintained at a temperature

of about 100 degrees F. during this application. The webbing is then passed through successive compartments 25 and 26 and an oven at temperatures of about 175 degrees F., 140 degrees F. in the respective ovens 25 and 26.

The relationship of the thinners to the binding materials, such as the oils and resins in the backsize and sandsize, is such as to minimize solvent action upon the underlying coat in the case of the sandsize, to avoid any softening or swelling of the binder coat. At the same time these materials should be of sufficient fluidity to seal up any pores which may have been caused by the evaporation of the solvent in the binder coat, or by the baking treatment to which the binder coat has been subjected.

The relationship of the ingredients to the thinner is further characterized by the ability of the thinner to maintain the solids substantially in perfect solution up to the end point of the evaporation of the thinners, to result in a film having the composite characteristics of all the residual ingredients uniformly blended.

Following the baking operation in the chambers 25 and 26, and before winding the composite article into rolls, the back surface of the webbing is sprayed with a mist of water in quantities just sufficient so that the paper does not cockle, the paper therefore being flexibilized by the moisture that is absorbed. The composite may then be formed into rolls and is then ready to be cut up into the final marketable article.

I have hereinbefore given specific examples of formulae which I prefer for purposes of making a sizing coat, binder coat, back-size or sand-size. In general, the proportions given may be varied and still obtain a high order of desirable results. The essential ingredients are the resinous components and fatty oils and these ingredients may be varied within limits more particularly set forth in the co-pending application of Carlton and Oakes, entitled Waterproof sandpaper and the method of making the same, filed on equal date with this application Serial No. 660,319. Accordingly, the resinous constituents and fatty oils may be varied within the following limits:

Resinous materials 12 to 39%; fatty oils from 81 to 50%; driers from .5 to 1%, and the balance up to about 40% of volatile thinners, the volatile thinners being variable, determined upon the point at which the composition is to be used, either as a paper sizing coat, binder coat, back-size or sand-size, further taking into account the nature of the backing material to be treated, the thickness of the binder coat that is desired, the size and nature of the abrasive particles.

In formulae C and F, I have referred to a phenol formaldehyde resin, specifying an "oil-reactive resin." Where the "oil-reactive resin" is used, it is preferred by me to use the oil reactive resin described in the aforementioned Carlton-Oakes application, and comprising a "phenol-fatty-oil-reactive resin," and where this form of oil reactive resin is used, it is submitted to polymerization in conjunction with a quality or the full amount of fatty oil designated in the various formulae. This combination of constituents is preferred by me as most suitable for practicing the process of making sandpaper in accordance with my invention hereinbefore described, in that the co-polymerization of the "phenol-fatty-oil-reactive resin" and the quantity of fatty oil designated lends itself peculiarly desirable to making sandpaper in accordance with my process in that

it permits a continuity of steps beginning with the application of the pre-size, followed by the application of the binder and, if desired, after application of the abrasive particles, the web carrying these layers may pass in a short time, directly and in a continuous operation, to the point where the back-size is applied and then to the point where the sandsize is applied.

Where I use the polymerization reaction product of a "phenol-fatty-oil-reactive resin" and the fatty oil in the volatile solvents, the web may pass through the pre-sizing operation and then to the point where the binder coat is applied with maximum speed, as only sufficient time necessary for volatilization of a portion of the solvent and aeration of the coating need expire and sufficient body will be given to the pre-sizing coat to permit it to directly pass to the point where the binder coat is applied, with the certainty that a proper relationship of the binder coat to the backing will be maintained, to avoid any undue starving of the binder coat to the quantity of abrasive particles deposited thereon.

It will be observed that from the disclosure made, I have provided compositions of particular utility in making waterproof sandpaper and a method for preparing waterproof sandpaper, having all the inherent advantages and desirable properties heretofore emphasized and which may serve to attain proper anchorage of the abrasive particles for maximum abrading efficiency, and uniformity of the end product and I consider the scope of my invention as pertaining to the compositions as residing in the provision of a composition particularly suitable for surface coating of the backing material used in making the sandpaper or the backing material having superimposed thereon a grit or layer of abrasive particles in which a proper balance of the vehicle is used, together with the resinous materials, in which the volatile components are so balanced that perfect solution of the waterproofing materials are maintained to the end point of evaporation, in the presence of porous solid materials, such as the backing, or in the presence of solid materials, such as the abrasive particles which are used. And I consider my invention to reside in the application of waterproofing materials to a backing material, or as a binder for an abrasive sheet or a size therefor, in which the inherent characteristics of the waterproofing materials in connection with the volatile solvent or a diluent are so balanced as to be characterized by perfect solution to the end point of evaporation, particularly in the presence of solid materials, or porous solid materials constituting either the backing material or the grit or layer of abrasive particles. And I further consider that the compositions herein disclosed and the method of producing the waterproof sandpaper herein described is characterized by the blend of the materials constituting the waterproofing material and the vehicle which, in the form of the final product, will result in an abrasive article of high efficiency, and with uniformity of characteristics, in that the waterproofing material will not flow from the grit or abrasive particles under the process of producing the final article, or cause any undue creeping of the binder in relation to the grit, in finally forming the article all of which characteristics hereinabove ascribed to my preferred form of binder which, for convenience, I term as "balanced composite" waterproofing material or binder. Where I use the term "bal-

anced composite" waterproofing material or binder in the claims, I mean to include within the scope thereof a binder having characteristics above mentioned specifically in this paragraph.

5 I also consider as novel in my invention the application of the grit in the manner set out and the removal of excess grit, together with the heating steps and subsequent treatment by sizing coats wherein the grit coated side of the sheet is maintained free of external pressure, thus preventing dulling of the finished article.

I also attribute the attainment of the novel features above described, permitting the continuity of operations, to the nature and character of the resinous and oily constituents in the volatile vehicle, these materials being balanced in perfect solution up to the end point of evaporation of the volatile vehicle, especially in the presence of the grit or layer of abrasive particles, and external pressure necessary for handling or uniting the coatings and which would otherwise disturb the efficiency of the abrading characteristics of the particles, is avoided.

I further consider that the novel characteristics of the method herein described for the formation of the waterproofing sandpaper resides in the control of the temperature and speed of volatilization of the volatile thinner or solvents, and that this includes the control of the temperature and the speed of volatilization above the dew point of the atmosphere in which the volatilization of the thinner is conducted and that this mode of operation materially contributes to the production of an abrasive product having high abrading efficiency and uniformity.

Having thus described my invention and illustrated its use, what I claim as new and desire to secure by Letters Patent, is:

1. The method of forming an abrasive article 40 including the steps of applying to a backing material a sizing coating of a "balanced composite" waterproofing material of a polymerized resin-oil complex homogeneously distributed in a volatile vehicle, aerating the backing so treated to 45 remove a portion of the volatile vehicle and oxidizing the sizing coat, applying a "balanced composite" waterproofing binder coating thereover comprising a resin-oil complex homogeneously, distributed in the volatile vehicle, depositing a 50 grit or layer of abrasive particles, diverting the abrasive particles from the binder coating in a direction away from the adhesive for removing the excess of the abrasive particles and then aerating to remove the volatile vehicle to the end 55 point of evaporation of the volatile vehicle, oxidizing the residuum in the presence of heat, the web being passed through the aeration and oxidizing steps under conditions leaving the abrasive surface exposed and free from external pressure until the coatings applied are set.

2. The method of forming an abrasive article including the steps of applying a rapidly setting sizing adhesive comprising a polymerized resin-oil complex to one side of a backing material, conducting the backing so as to aerate the sizing adhesive, then immediately applying an adhesive formed of a "balanced composite" waterproofing material comprising a polymerized oil-resin complex in plastic state to the sized 65 surface of said backing and while said adhesive is still plastic applying a grit or layer of abrasive particles upon the adhesive coated side of said backing, and diverting the abrasive from the adhesive coated side in a direction away 70 from the adhesive for removing the excess of

said particles, then continuously feeding the backing so prepared and subjecting same to heat without external pressure upon the abrasive coated surface from the point of deposition of grit until the adhesive is set.

3. The method of forming an abrasive article including the steps of applying a rapidly setting sizing adhesive comprising a polymerized resin-fatty-oil complex to one side of a backing material, conducting the backing so as to aerate the sizing adhesive, then immediately applying an adhesive formed of a "balanced composite" waterproofing material comprising a polymerized resin-fatty-oil complex in plastic state to the sized surface of said backing and while said adhesive is still plastic applying a grit or layer of abrasive particles upon the adhesive coated side of said backing, and diverting the abrasive from the adhesive coated side in a direction away from the adhesive for removing the excess of said particles, then continuously feeding the backing so prepared while applying a grit sizing coat and subjecting the article to heat without external pressure upon the abrasive coated surface from the point of deposition of the grit until the adhesive is set.

4. The method of forming an abrasive article including the steps of continuously and progressively applying to a carrier successive coats formed of a "balanced composite" waterproofing material of a polymerized "phenol-fatty-oil-reactive resin" and fatty oil in a volatile vehicle, each of the successive coats being subjected to aeration and oxidation during intervals between the application of the coats, one of said coatings being followed by a deposition of a grit or layer of abrasive particles while the coating is in a plastic state.

5. In the method of forming an abrasive article, the steps which include applying a sizing coat to a backing material comprising a polymerized reaction product of a "phenol-fatty-oil-reactive resin" and a fatty oil in a volatile vehicle, aerating the coating so deposited upon the backing, overlying a "balanced composite" waterproofing binder coat comprising a polymerized reaction product of a "phenol-fatty-oil-

reactive resin" and a fatty oil in a volatile vehicle, depositing a grit or layer of abrasive particles, aerating the backing material and its coatings to separate a portion of the volatile vehicle by disposing the web to expose the surface coating thereof without external pressure, oxidizing the last mentioned coating in the presence of heat while oxidizing the surface thereof without external pressure upon the abrasive coated surface from the point of deposition of the grit or layer of abrasive particles until the binder coat is set.

6. In the method of forming an abrasive article in the nature of sandpaper, the steps which include continuously and progressively applying successive coats formed of a "balanced composite" waterproofing material to one side of a backing material in successive coatings, said material being formed of a polymerized resin-fatty oil complex homogeneously distributed in a volatile vehicle, each of the successive coats being subjected to aeration and oxidation during the application of the coats, the period of operation for the first of said coats partially setting the polymerized fatty oil resin complex, one of said coatings being followed by a deposition of the grit or layer of abrasive particles while the coating is in a plastic state.

7. In the method of forming an abrasive article in the nature of sandpaper, the steps which include continuously and progressively applying successive coats formed of a "balanced composite" waterproofing material to one side of a backing material in successive coatings, said material being formed of a polymerized "phenol-fatty-oil-reactive-resin" and a fatty oil homogeneously distributed in a volatile vehicle, each of the successive coats being subjected to aeration and oxidation during intervals between the application of the coats, the period of operation for the first of said coats partially setting the said polymerized resin and oil, one of said coatings being followed by a deposition of the grit or layer of abrasive particles while the coating is in a plastic state.

BYRON J. OAKES.